

## UNITED STATES PATENT OFFICE

2,420,953

## LUBRICANT

Russell A. Hunt, Jr., Hammond, Ind., assignor to  
 Standard Oil Company, Chicago, Ill., a corpora-  
 tion of Indiana

No Drawing. Application August 19, 1944,  
 Serial No. 550,305

15 Claims. (Cl. 252—49.9)

1

This invention relates to improvements in lub-  
 bricants and more specifically to improvements in  
 lubricants which come in contact with copper  
 surfaces such as ice machine lubricants.

In the lubrication of certain types of machin-  
 ery in which the lubricant comes in contact with  
 copper parts of such equipment, it has been ob-  
 served that a phenomenon known as "copper plating"  
 takes place. This phenomenon occurs partic-  
 5 ularly in the lubrication of refrigerators or ice  
 machines. In the lubrication of such equipment  
 the oil employed comes in contact with the cop-  
 per coils and other parts of the equipment in  
 which copper is employed. Copper plating of the  
 nature herein referred to is the phenomenon in  
 which copper is removed from certain parts of  
 the equipment and deposited in other parts  
 thereof. Thus in refrigeration systems, for ex-  
 ample, copper is removed from elements such  
 as the copper tubing and deposited on the parts  
 of the system which are formed of some metal  
 other than copper or its alloys such as the steel  
 or other ferrous metal parts of the equipment.  
 Usually the deposit of copper takes place on  
 moving parts of the system such as on pistons  
 and/or valves and results frequently in serious in-  
 terference in operation of the machinery. This  
 phenomenon of copper plating is associated with  
 the lubricating oil employed for the lubrication  
 of moving parts of such equipment. The reason  
 for this copper plating is not completely under-  
 stood. However, the fact remains that it does  
 occur even though highly refined lubricating oils  
 are usually employed in the lubrication of such  
 equipment.

It is therefore an object of this invention to  
 provide a lubricant which will prevent copper  
 plating in equipment in which such lubricant is  
 employed. Another object of the present inven-  
 tion is to provide an improved refrigerator lubri-  
 cant which will prevent copper plating.

Still another object of the invention is to pro-  
 vide a method of preventing copper plating in  
 the lubrication of equipment in which copper or  
 copper alloys are employed.

I have discovered that the foregoing objects  
 can be attained by lubricating systems in which  
 copper and/or copper alloys are employed with  
 a highly refined hydrocarbon oil, particularly a  
 synthetic hydrocarbon oil containing small

2

amounts of a copper deactivator and preferably  
 a phenyl-alpha-naphthylamine.

While the present invention is applicable to  
 any highly refined hydrocarbon oil which is sus-  
 ceptible to copper plating, it is particularly ap-  
 plicable to synthetic hydrocarbon oils, and es-  
 pecially to a mono-olefin polymer having a Say-  
 bolt Universal viscosity at 100° F. of from about  
 50 seconds to about 400 seconds or higher de-  
 pending upon the type of equipment to be lubri-  
 cated. This synthetic oil is preferably an olefin  
 hydrocarbon polymer resulting from the poly-  
 merization of low molecular weight mono-olefinic  
 hydrocarbons or isomono-olefinic hydrocarbons  
 15 or mixtures thereof such as propylene, butylenes  
 and amylenes. These polymers or copolymers  
 can be obtained by the polymerization of these  
 olefins or mixtures of olefins in the presence of  
 20 a catalyst such as sulfuric acid, phosphoric acid,  
 boron fluoride, aluminum chloride or similar  
 halide catalysts of the Friedel-Crafts type. A  
 suitable synthetic oil is one obtained by poly-  
 merizing in the liquid phase a hydrocarbon mix-  
 25 ture containing mono-olefins and iso-olefins such  
 as butylene and isobutylene at a temperature of  
 from about 50° F. to about 100° F. in the presence  
 of a metal halide catalyst of the Friedel-Crafts  
 30 type, such as, for example, boron fluoride, alu-  
 minum chloride and the like. A suitable source  
 of low molecular weight olefinic hydrocarbons  
 suitable for this purpose is a hydrocarbon mixture  
 35 containing isobutylene, butylene and butanes re-  
 covered from petroleum gases, especially those  
 gases produced in the cracking of petroleum oils  
 in the manufacture of gasoline.

Another suitable polymer is that obtained by  
 polymerizing at a temperature of from about 50°  
 F. to about 110° F. in the liquid phase a hydro-  
 40 carbon mixture comprising substantially C<sub>3</sub> hy-  
 drocarbons in the presence of an aluminum chlo-  
 ride complex catalyst. The catalyst is prefer-  
 ably prepared by heating aluminum chloride with  
 iso-octane. The propylene polymer so obtained  
 45 can be fractionated to obtain a fraction having  
 the desired viscosity range.

Suitable copper deactivators which can be em-  
 ployed in the present invention are the reaction  
 products of aromatic ortho hydroxy aldehydes,  
 such as 2-hydroxybenzaldehyde, 2-4-dihydroxy-  
 50 benzaldehyde, 2 - hydroxy - 3 - methoxybenzalde-

hyde, etc. with polyamines, particularly an aliphatic polyamine containing at least two primary amino nitrogen atoms, such as methylenediamine, ethylene diamine, diethylene triamine, 1-10-decylene diamine, triethylene tetramine, propylene diamine, tetraethylene pentamine, etc. Suitable copper deactivators also are those obtained by reacting an ortho hydroxy aromatic ketone with an aliphatic polyamine containing at least two primary amino groups. Specific examples of such compounds are di-2-hydroxy acetophenone ethylene diamine, di-2-hydroxy propiophenone ethylene diamine, di-2-hydroxy-5-methylacetophenone - 1,3 - propylene diamine, etc. Other copper deactivators which can be employed in the present invention are the reaction products of diacyl compounds and primary amines such as dibenzoyl acetonyl ethylene diamine and diacetyl acetonyl ethylene diamine; hydroxy aromatic aldoximes and ketoximes such as ortho hydroxybenzaldoxime, ortho hydroxyacetophenone, etc. While compounds of the foregoing type are all active metal deactivators, particularly copper deactivators, they all are not equally effective. The copper deactivator can be employed in amounts of from about 0.001% to about 2% and preferably from about 0.005% to about 0.05%.

In addition to the metal deactivator, the lubricant composition of the present invention preferably also contains a small amount—namely, from about 0.001% to about 2% and preferably from about 0.01% to about 0.5% of a phenyl-alpha-naphthylamine.

When desired the lubricant can contain other additives such as, for example, from about 0.5% to about 3% of a film strengthening additive, e. g. tricresyl phosphate and the like.

In order that the present invention may be more fully appreciated and understood, the same will be described in connection with an ice machine oil composition although it is to be understood that this is given merely by way of illustration and not to be construed as a limitation upon the scope of the present invention. An ice machine oil comprising a butylene polymer having a Saybolt Universal viscosity at 100° F. of about 50 seconds was compounded with 0.02% of a copper deactivator obtained by reacting salicylal with a polyamine and 0.01% of phenyl-alpha-naphthylamine. The ice machine oil also contained in addition to the aforementioned additives 1% of tricresyl phosphate to increase the film strength of the oil. The resistance to copper plating of this oil was compared with the resistance to copper plating of the same butylene polymer containing only the copper deactivator and another sample of the oil containing only phenyl-alpha-naphthylamine. In determining the resistance to copper plating or the "copper susceptibility" of the various oils 25 cc. of the oil to be tested in contact with 6½ feet of clean, bright, No. 18 gauge copper wire is heated at 200° F. A sample of oil is then mixed with an equal portion of diphenylthiocarbazone (dithizone) solution to determine the presence of copper in the solution, a purple color indicating that copper is present. Samples of the oil are taken, tested at 2 hours, 6 hours and 24 hours and every 24 hours thereafter until a positive copper test is obtained. The "copper life" is the time required for a positive copper test by this method.

The dithizone solution used to determine the presence of copper in the oil is prepared by dis-

solving 50 mg. of diphenylthiocarbazone in one liter of carbon tetrachloride. Since the dithizone reagent is extremely sensitive to light, the reagent must be kept in a dark bottle under refrigeration. The effect of the copper deactivator in preventing copper plating is demonstrated by the data in Table I. The synergistic effect of the combination of a metal deactivator and a phenyl-alpha-naphthylamine is illustrated by the following copper susceptibility data in Table II.

Table I

|    | Oil                           | Additive                                            | Hours to show Positive Copper Test |
|----|-------------------------------|-----------------------------------------------------|------------------------------------|
| 20 | Butylene polymer <sup>1</sup> | None                                                | 6                                  |
|    | Do. <sup>1</sup>              | 1.0% tricresyl phosphate                            | 24                                 |
|    | Do. <sup>1</sup>              | 0.02% copper deactivator <sup>2</sup>               | 72                                 |
| 25 | Butylene polymer <sup>2</sup> | None                                                | 6                                  |
|    | Do. <sup>2</sup>              | 0.02% copper deactivator + 1.0% tricresyl phosphate | 200+                               |
|    | Butylene polymer <sup>3</sup> | None                                                | 6                                  |
| 30 | Do. <sup>3</sup>              | 0.02% copper deactivator + 1.0% tricresyl phosphate | 200+                               |
|    | Butylene polymer <sup>4</sup> | None                                                | 6                                  |
|    | Do. <sup>4</sup>              | 0.02% copper deactivator + 1.0% tricresyl phosphate | 200+                               |

Table II

|    | Oil                           | Additive                                                   | Hours to show Positive Copper Test |
|----|-------------------------------|------------------------------------------------------------|------------------------------------|
| 35 | Butylene polymer <sup>1</sup> | None                                                       | 6                                  |
|    | Do. <sup>1</sup>              | 0.02% copper deactivator <sup>3</sup>                      | 72                                 |
|    | Do. <sup>1</sup>              | 0.01% phenyl-alpha-naphthylamine                           | 2                                  |
| 40 | Do. <sup>1</sup>              | 0.02% copper deactivator + 0.0% phenyl-alpha-naphthylamine | 96                                 |
|    | Butylene polymer <sup>1</sup> | None                                                       | 6                                  |
|    | Do. <sup>1</sup>              | 0.02% copper deactivator + 0.0% phenyl-alpha-naphthylamine | 72                                 |

<sup>1</sup> Saybolt Universal viscosity at 100° F. = 50 secs.

<sup>2</sup> Saybolt Universal viscosity at 100° F. = 100 secs.

<sup>3</sup> Saybolt Universal viscosity at 100° F. = 200 secs.

<sup>4</sup> Saybolt Universal viscosity at 100° F. = 400 secs.

<sup>5</sup> Reaction product of salicylal and triethylene tetramine.

To facilitate solution of the additives in the hydrocarbon oil, it is frequently advisable to incorporate the additives in the oil in the presence of an aromatic solvent. A suitable solvent for this purpose is a fraction high in aromatics obtained by the catalytic conversion of petroleum naphtha in the presence of a dehydrogenating catalyst and preferably in the presence of hydrogen. The product of this conversion is a mixture of reformed naphtha suitable for gasoline of high knock rating and heavier hydrocarbons boiling largely above the boiling point of the naphtha charged. This reaction product boiling within the range of about 425° F. to about 600° F. is high in aromatics and contains liquid derivatives of naphthalene. This fraction is known as hydroformer bottoms. While I prefer to use these hydroformer bottoms as the solvent in the preparation of the herein-described lubricants, other suitable solvents can, of course, be used.

While I have described my invention with particular reference to refrigerator or ice machine lubricants, it is to be understood that the invention is not limited to this particular type of lubricant but is applicable to any lubricant susceptible to cause copper plating when used in the presence of copper or copper alloys.

I claim:

1. A hydrocarbon oil composition resistant to copper plating comprising a hydrocarbon oil normally susceptible to cause copper plating in the presence of a copper-containing metal, a copper deactivator and tricresyl phosphate, said copper deactivator and said tricresyl phosphate being used in small but sufficient quantities to inhibit the copper plating by said hydrocarbon oil said copper deactivator being the reaction product of an aliphatic polyamino compound having at least two primary amino nitrogen atoms and an aromatic compound selected from the class consisting of aromatic ortho hydroxy aldehydes and ortho hydroxy aromatic ketones.

2. A hydrocarbon oil composition as described in claim 1 in which from about 0.001% to about 2% of the copper deactivator and from about 0.5% to about 3% of the tricresyl phosphate are employed.

3. A hydrocarbon oil composition as described in claim 1 containing from about 0.01% to about 0.5% of a phenyl alpha-naphthylamine.

4. A hydrocarbon oil composition as described in claim 1 in which the metal deactivator is the reaction product of an aromatic ortho hydroxy aldehyde and an aliphatic polyamino compound having at least two primary amino nitrogen atoms.

5. A hydrocarbon oil composition as described in claim 1 in which the copper deactivator is the reaction product of ortho hydroxy benzaldehyde and an aliphatic amine having at least two primary amino nitrogen atoms.

6. A hydrocarbon oil composition as described in claim 1 in which the copper deactivator is the reaction product of an ortho hydroxy aromatic ketone and an aliphatic polyamine containing at least two primary amino nitrogen atoms.

7. A hydrocarbon oil composition which does not cause copper plating in the presence of a copper-containing metal comprising a synthetic hydrocarbon oil obtained by the polymerization of monoolefins, and which normally is susceptible to cause copper plating in the presence of a copper-containing metal, a copper deactivator and tricresyl phosphate, said copper deactivator and said tricresyl phosphate being used in small but sufficient quantities to inhibit the copper plating by said synthetic hydrocarbon oil, and said copper deactivator being the reaction product of an aliphatic polyamino compound having at least two primary amino nitrogen atoms and an aromatic compound selected from the class consisting of aromatic ortho hydroxy aldehydes and ortho hydroxy aromatic ketones.

8. A hydrocarbon oil composition as described in claim 5 in which the synthetic hydrocarbon oil is a butylene polymer having a Saybolt Universal viscosity at 100° F. of from about 50 seconds to about 400 seconds.

9. A hydrocarbon oil composition as described in claim 5 in which the synthetic hydrocarbon oil is a propylene polymer having a Saybolt Universal viscosity at 100° F. of from about 50 seconds to about 400 seconds.

10. A hydrocarbon oil composition as described in claim 5 in which the metal deactivator is the reaction product of an aromatic ortho hydroxy

aldehyde and a polyamino compound having at least four nitrogen atoms of which at least two are primary amino nitrogen atoms.

11. A hydrocarbon oil composition as described in claim 5 in which the copper deactivator is the reaction product of ortho hydroxy benzaldehyde and an alkylene amine having at least four nitrogen atoms of which at least two are primary amino nitrogen atoms.

12. A hydrocarbon oil composition as described in claim 5 in which the copper deactivator is the reaction product of an ortho hydroxy aromatic ketone and an aliphatic polyamine containing at least two primary amino nitrogen atoms.

13. A hydrocarbon oil composition which does not cause copper plating in the presence of a copper-containing metal comprising a mono-olefin polymer oil having a Saybolt Universal viscosity at 100° F. of from about 50 seconds to about 400 seconds and normally susceptible to cause copper plating in the presence of copper-containing metal, from about 0.005% to about 0.05% of the reaction product of ortho hydroxy benzaldehyde and an aliphatic polyamine containing at least two primary amino nitrogen atoms, from about 0.01% to about 0.5% of a phenyl-alpha-naphthylamine and from about 0.5% to about 3% of tricresyl phosphate.

14. The method of preventing copper plating in a system containing copper-containing metal lubricated with a hydrocarbon oil comprising lubricating said system with a hydrocarbon oil composition comprising a hydrocarbon oil normally susceptible to cause plating in the presence of a copper-containing metal, a copper deactivator and tricresyl phosphate in small but sufficient quantities to substantially inhibit copper plating of said hydrocarbon oil said copper deactivator being the reaction product of an aliphatic poly-amino compound having at least two primary amino nitrogen atoms and an aromatic compound selected from the class consisting of aromatic ortho hydroxy aldehydes and ortho hydroxy aromatic ketones.

15. The method described in claim 12 in which the hydrocarbon oil is a mono-olefin polymer oil having a Saybolt Universal viscosity at 100° F. of from about 50 seconds to about 400 seconds and which is normally susceptible to cause copper plating in the presence of a copper-containing metal and in which the copper deactivator is a reaction product of an aromatic ortho hydroxy aldehyde and an aliphatic polyamine containing at least two primary amino nitrogen atoms.

55 RUSSELL A. HUNT, JR.

#### REFERENCES CITED

The following references are of record in the file of this patent:

#### 60 UNITED STATES PATENTS

| Number       | Name                 | Date          |
|--------------|----------------------|---------------|
| 2,352,462    | Weiss et al. -----   | June 27, 1944 |
| 2,352,164    | Burnham -----        | June 27, 1944 |
| 65 2,351,380 | White -----          | June 13, 1944 |
| 2,270,577    | Bergstrom -----      | Jan. 20, 1942 |
| 2,239,501    | Frolich et al. ----- | Apr. 22, 1941 |
| 2,143,566    | Moser -----          | Jan. 10, 1939 |